

July 6, 1926.

1,591,372

D. W. GAFVERT ET AL

HOLLOW STEEL BALL AND METHOD OF MAKING IT

Filed Oct. 23, 1925

Fig. 1.



Fig. 2.



Fig. 3.



Fig. 4.



Fig. 5.



Fig. 6.



Fig. 7.



Fig. 8.



Fig. 9.



Inventors

DAVID W. GAFVERT,  
GUNARD O. CARLSON,

By Jack Richmond

Attorney

Patented July 6, 1926.

## UNITED STATES PATENT OFFICE.

DAVID W. GAFVERT AND GUNARD O. CARLSON, OF EASTON, PENNSYLVANIA, ASSIGNEES TO WILLIAM WHARTON JR. & CO., INCORPORATED, OF EASTON, PENNSYLVANIA, A CORPORATION OF PENNSYLVANIA.

## HOLLOW STEEL BALL AND METHOD OF MAKING IT.

Application filed October 23, 1925. Serial No. 64,352.

Our invention is concerned more particularly with the production of balls for use as check valves in pumps, rams and other hydraulic machinery. Check valves of this type range from very small sizes to relatively large sizes. It has been customary to press the smaller sizes from sheet metal and to either cast the larger sizes or to fabricate them from two or more sections. These practices are costly and the products are open to the objections of flashing, subnormal or abnormal weight, improper balance and generally to the lack of true spherical quality so necessary to meet the efficiency demanded of valves of this type.

We propose to obviate the aforementioned objections by providing a hollow steel ball forged from a billet whereby we lessen the cost of production and insure products of uniformly high rating as regards distribution of weight, strength, perfection of shape, smoothness of surface, and overall efficiency to meet the demands of service.

The nature, characteristic features and scope of the invention will more readily be understood from the following description taken in connection with the accompanying drawings, forming a part hereof, wherein—

Figure 1 is a sectional view of the billet 30 positioned for piercing;

Fig. 2 is a sectional view showing the forging resulting from the operation, Fig. 1;

Fig. 3 is a similar view of the forging after cropping;

Figs. 4, 5 and 6 illustrate the development of necking;

Fig. 7 illustrates the condition of the work after the removal of the neck;

Fig. 8 illustrates the next phase of filling 40 the void established by closing in or necking; and

Fig. 9 is a sectional view of the finished ball.

According to our invention we start with 45 a billet 5 of round or polygonal section. This is heated to forging or working temperature and arranged for piercing in a die 6. The cavity of the latter is cylindrical and semi-circular with respect to the walls 7 and bottom 8 the latter being interrupted by an axial opening 9. The die 6 in co-operation

with a piercing tool 10 produces the hollow forging shown in Fig. 2. An important feature of that forging is the presence at the closed or rounded end of a boss or projection 11, for holding and manipulating the forging throughout the remaining operations of cropping, closing in or necking and plugging.

Fig. 3 represents the forging after its 60 ragged or rough end 12 has been cropped.

Figs. 4, 5 and 6 show formative stages leading to the development of the neck 13, Fig. 6. This operation is performed in a manner well known and not requiring illustration.

The next operation is to remove the neck to produce the article, Fig. 7. In this state there is a void 14 which makes for unbalanced weight. We eliminate this condition 70 by drilling and tapping co-extensive with the void and filling the drilled hole with a screw plug 15. Before inserting the plug use is made of the drilled opening to center the article and cut off the boss or projection 11. 75 The finished article is shown in Fig. 9.

Having described our invention, we claim:

1. The method of producing articles of the nature indicated which consists in piercing a billet to produce a hollow structure having a substantial area of the shape of the finished article, closing the open end by working, removing the neck resulting from working, and unifying the distribution of 85 weight by drilling and plugging the necked area.

2. The method of producing articles of the nature indicated which consists in piercing a billet to produce a hollow structure 90 having a substantial portion of the shape of the finished article and having a centering boss or projection, closing the open end by working, removing the neck resulting from working, drilling and tapping the necked area, removing the centering boss, and plugging the necked area.

In testimony whereof we affix our signatures.

DAVID W. GAFVERT.  
GUNARD O. CARLSON.